

## UNITED STATES PATENT OFFICE

2,384,837

SULPHONIC ACIDS OF THE 5-OXO  
IMIDAZOLINE SERIES

Oskar Huppert, Chicago, Ill.

No Drawing. Application March 3, 1941,  
Serial No. 381,545

10 Claims. (Cl. 8—127.5)

This invention relates to new sulphonic acids, their salts and esters, particularly to artificial protein fibers containing the same whereby improvements in wet strength, lustre and resistance to swelling result.

The new compounds have in their acid form the general formula:



wherein R indicates hydrogen, alkyl, aryl-alkyl or a heterocyclic radical and x indicates a number from 0 to 287. (For the specific term R see: "Das Protein und seine stereoisomeren Modifikationen. Chemische Physik und Biochemie," page 20 17, picture IV, by Huppert, Vienna 1933, Chemical Abstracts 23, 3244.)

In my United States Patent Number 2,112,210 and in my co-pending application Serial Number 378,774, filed February 13, 1941, I described thiourea disulphides, substituted in the nucleus in position 3 and 5, prepared from proteins and alpha amino acids. As disclosed in said patent these disulphides may be formed by treating the starting amino compounds with carbon disulphide at an hydroxyl ion concentration not exceeding that of a solution of calcium hydroxide in water and oxidizing the thus sulphurized material to form the disulphide.

I have now found that these compounds can be converted into derivatives of the hydantoin-2 sulphonic acid. This process consists generally in oxidizing the disulphide group to the sulphonic group with hydrogen peroxide or halogen. The following chemical reaction takes place:



The compounds of the present invention can also be considered as derivatives of imidazoline and are 5-oxo imidazoline sulphonic acid-2 compounds substituted in the 1 and 4 positions.

In the following formula the Formula A shows the numbering for the hydantoin ring and Formula B shows the numbering when considering the ring as the imidazoline.



(A)



(B)

The compounds of the present invention possess very resistant sulphonic groups and have specific detergent and textile finishing properties. They show a great affinity for protein fibers such as artificial fibers, wool, and the like and increase the elasticity and flexibility of such fibers. For instance, if artificial protein fibers which have been prepared by first spinning into the coagulating bath, stretching, hardening, washing, impregnating with quaternary ammonium compounds over-baking and drying, are treated with the compounds of the present invention the relatively brittle fibers are rendered much more flexible and useful.

15 Instead of impregnating formed fibers with solutions of the sulphonic acids of the present invention fibers containing the protein disulphide prepared according to United States Patent No. 2,112,210 may be treated with hydrogen peroxide to convert the protein thiourea disulphides into the corresponding sulphonic acids in situ. By such a procedure the wet strength of the fiber is increased and the swelling decreased.

The salts of these sulphonic acids, particularly 25 those of the alkali-, aluminum-, zinc-, chrome-metals, amine bases can be prepared in the usual manner.

The sulphonic acids and their salts are all soluble in water and are capillary active and hence 30 these products and their esters with high fatty alcohols can be used as detergents, as protective colloids, as wetting, dispersing emulsifying and softening agents, for improving dye fastness.

Certain sulphonic acids, manufactured from 35 alpha amino acids, for instance, from tyrosine, according to this invention, are excellent edible dyes, soluble in water and alcohol, and can be used in the food and baking industry. (The dough, for instance, can be coloured with these products as they are yellow like the egg-yolk.) Furthermore these dyes are useful for colouring drugs, cosmetics and fats.

These compounds can be used in the textile, 45 leather, fat and pharmaceutical industry and as insecticides and fungicides.

Especially these sulphonic acids can be used as dyestuff-preparations to change the fibers in such a manner that they can be coloured with special dyestuffs.

## Example 1

50 10 liters water are poured over 1000 g. technical gelatine and the mixture is allowed to stand and swell over night. One obtains thereby a gelatine 55 solution of 10%. 70 g. lime hydrate, dispersed in water, are added. The mixture is heated for one hour under vigorous stirring and then filtered. 64 cc. carbon disulphide are added under vigorous stirring at a temperature of 40° C. and 60 sulphurated for half an hour. The excess of the

carbon disulphide is removed by heating to 80° C. One obtains a solution of "Leukothiogelatine." Then 70 g. manganese dioxide are added under vigorous stirring and boiled for about 20 to 30 minutes until the solution becomes blood-red with a shine into purple. The solution is now allowed to stand, decanted of the manganese dioxide and filtered. Afterwards 15.5 g. sulphuric acid are added to the red solution, care being taken against foaming. The colour turns from red to yellow. One tries with Congo paper for the blue colour. This reaction takes place at about the boiling temperature. The gypsum is then filtered after 4 hours. Now 3 cc. acetic acid (80%) and 2500 cc. hydrogen peroxide (3%) are successively added to the solution and boiled for half an hour. By evaporation to dryness on a drum dryer one obtains the sulphonic acid of the hydantoin.

*Example 2*

181 g. tyrosine are dissolved in 1200 cc. water. 80 g. sodium hydroxide are added and the solution is warmed to 40° C. and filtered. 80 cc. carbon disulphide are added to the solution and boiled under reflux for one hour with agitation at 45° C. Thereafter the excess of the carbon disulphide is removed and the solution is heated to 70° C. Now 70 g. manganese peroxide are added and the solution is held under stirring at 90° C. for 15 minutes. The manganese peroxide is filtered and the orange coloured solution of the 5 (4 oxybenzyl) 2 thiohydantoin 3 (4 oxybenzyl) acetic acid disulphide is obtained as the sodium salt. 80 g. sulphuric acid and 40 g. acetic acid (80%) are added to the solution which is then warmed to 40° C. Now 140 cc. hydrogen peroxide (30%) are added to the solution, which is warmed slowly until boiling and then boiled for 10 minutes. By evaporation one obtains the 2 sulphonic acid of the 5 p.oxybenzyl-hydantoin 3 p.oxybenzyl acetic acid in crystals, after one has extracted the residue with boiling alcohol.

*Example 3*

Artificial fibers, spun from mixtures of casein thiohydantoin-disulphide and urea are soaked at a temperature of 40° C., after hardening, washing, impregnating with quaternary ammonium compounds, drying and baking, in an aqueous bath containing 5% by weight of the aluminum salt of the hydantoin-gelatose-sulphonic-acid of Example 1. After 10 minutes the fibers are taken out of the bath and dried. They have been prepared in such a manner that they have the affinity to be dyed with palatine-dyestuffs.

It will be understood that the detailed procedures described are capable of wide variations and modifications without departing from the spirit of this invention.

Having now particularly described and ascertained the nature of my invention and in what manner the same is to be performed, I declare that what I claim is:

1. The process which comprises oxidizing disulphides selected from the class having the formula



with hydrogen peroxide to form the sulphonic acids having the formula



10 in which R is a group selected from the class consisting of hydrogen atoms, aliphatic, aliphatic-aromatic and heterocyclic radicals found in  $\alpha$ -amino acids, and x is a number from 0 to 287.

15 2. The compound of the following formula, prepared from tyrosine:



20 3. A protein fiber containing a sulphonic compound selected from the class consisting of sulphonate acids obtainable by oxidizing with hydrogen peroxide the disulphide formed by treating an amino-compound selected from the class consisting of proteins and alpha-amino acids with carbon disulphide at a hydroxyl ion concentration not exceeding that of an aqueous solution of calcium hydroxide and oxidizing the thus sulphurized compound to form the disulphide, and salts and esters of said sulphonate acids.

25 35 4. A protein fiber containing the sulphonate acid oxidation product resulting from treating a thiohydantoin disulphide with hydrogen peroxide.

5. A protein fiber containing the sulphonate acid oxidation product resulting from treating a thiohydantoin protein disulphide with hydrogen peroxide.

40 6. A protein fiber according to claim 3 in which the disulphide is prepared from alpha-amino acids.

45 7. The process of treating protein fibers which comprises incorporating in the fiber a sulphonate compound selected from the class consisting of sulphonate acids obtainable by oxidizing with hydrogen peroxide the disulphide formed by treating amino compounds selected from the class consisting of proteins and amino acids with carbon disulphide at a hydroxyl ion concentration not exceeding that of a solution of calcium hydroxide and oxidizing the thus sulphurized product to form the disulphide, and salts and esters of said sulphonate acids.

50 8. Compounds selected from the class consisting of (1) sulphonate acids having the formula



55 65 in which R is a group selected from the class consisting of hydrogen atoms, aliphatic, aliphatic-aromatic and heterocyclic radicals found in  $\alpha$ -amino acids and x is a member from 0 to 287, (2) salts thereof, and (3) esters thereof.

70 9. The compounds of claim 8 in which x is 0.

10. The compounds of claim 8 in which x is greater than 0.

OSKAR HUPPERT.